

## UNITED STATES PATENT OFFICE

2,178,744

## COLORATION OF TEXTILE MATERIALS

George Holland Ellis and Charles Finley Topham,  
Spondon, near Derby, England, assignors to  
Celanese Corporation of America, a corpora-  
tion of Delaware

No Drawing. Application October 20, 1937, Se-  
rial No. 170,053. In Great Britain November 9,  
1936

7 Claims. (Cl. 8—24)

This invention relates to improvements in the coloration of textile materials and particularly to improvements in the coloration of mixed textile materials containing filaments or fibres of organic derivatives of cellulose and other filaments or fibres, for example cotton fibres.

According to the present invention mixed textile materials containing filaments, yarns or the like of organic derivatives of cellulose and other filamentary constituents are solid or cross-dyed by impregnating the materials with diazotisable bases, including diazotisable dyestuffs, which, when diazotised and coupled, form dyestuffs both for the organic derivative of cellulose constituents and for the other constituents, and then effecting diazotisation and coupling of the diazotised bases. Preferably the coupling components for the organic derivative of cellulose constituents are incorporated in the materials before diazotisation. With suitable components, coupling to form the dyestuff for the organic derivative of cellulose materials may take place in the cold, e. g. simultaneously with diazotisation. In other cases it may be desirable to treat the materials at an increased temperature, e. g. 60 to 80° C., in the presence of the coupling component after formation of the dyestuff for the cotton or other constituent has been effected at a lower temperature, e. g. 10 to 20° C.

While it is preferable to incorporate the coupling component for the organic derivative of cellulose constituent in the materials before diazotisation this is not essential and if desired the whole of the coupling component or components may be introduced into the fabric or other material after diazotisation. In this case boric acid or other suitable buffering agent may be introduced into the medium containing the coupling component, after cold coupling of the diazo compound on the cotton fibre has been effected, in order to assist the coupling of the diazo compound on the cellulose acetate or other organic derivative of cellulose filaments during a treatment at raised temperature.

The following are examples of the dyeing of mixed fabrics according to the process of the present invention:—

*Example 1*

A cellulose acetate-cotton woven fabric is introduced into a dyebath containing about 3% of a 10% paste containing 1-amino-3-methoxy benzene-4-azo-dimethylaniline, 0.4% of a 10% paste containing 4-nitro 2-methoxy amino benzene, about 10% of Chlorazol Black B. H. (Color

Index No. 401), about 1% of naphthol A. S., 0.3% of caustic soda and 1% of boric acid. The dyebath ratio is about 30:1 and the initial temperature is 45° C., the temperature being raised during an hour to about 80° C. Two additions of 5 50% of Glauber's salt are made during the treatment. After this treatment the fabric is washed off and diazotised at 10°-20° C. for 30 minutes in a 30:1 bath containing about 5% of sodium nitrite and 20% of formic acid. It is then washed off and introduced into a 30:1 bath containing about 1% of naphthol A. S. and 0.3% caustic soda and is worked first for about 30 minutes at a temperature of 10-15° C. to form the cotton dyestuff and then for a further 30 minutes at a temperature of 75° C. to form the cellulose acetate dyestuff. The fabric is then introduced into a cold soap bath having a soap concentration of about 0.25% and containing about 3% of soda ash, the temperature being raised to 75° C. 20 during about half an hour. The fabric is then washed off and dried.

The proportions of reagents given above are all based on the weight of the fabric except where otherwise stated.

*Example 2*

A mixed cellulose acetate viscose fabric is dyed in a bath containing 10% of ortho-methoxy benzene azo- $\alpha$ -naphthylamine and 4% of diazo fast yellow 3GL, exhaustion being assisted, if necessary, by the addition of salt. The material is then diazotised in the cold, rinsed and treated in a bath containing 2% of  $\beta$ -naphthol at room temperature, the temperature being gradually raised to about 60° C.

In this manner a dyed mixed fabric is obtained in which the cellulose acetate yarn is dyed a deep purple and the viscose yarn a reddish orange.

*Example 3*

A mixed cellulose acetate viscose fabric is dyed in a bath containing the following constituents:

|                                           | Per cent |
|-------------------------------------------|----------|
| Fast red RL base                          | 1        |
| Naphthol AS.LT                            | 2        |
| Sodium hydroxide                          | 0.5      |
| Chlorazol Black BH. (Color Index No. 401) | 10       |

The alkali is buffered with boric acid or glucose and the material is treated for about an hour at 75 to 80° C. with the addition of 50% of Glauber's salt to increase the exhaustion of the cotton color. After rinsing the material is introduced into a 15:1 bath containing 5% of sodium

55

- nitrite and 20% of formic acid and worked cold for 30 minutes. Diazotisation of the bases and coupling on the cellulose acetate take place in this bath, a deep red color being developed after about 30 minutes. The material is then rinsed and introduced into a fresh bath, containing one gram per litre of soda ash and 1% of naphthol AS.LT dissolved in 0.25% of caustic soda, to complete coupling on the viscose.
- 10 In this manner a dyed mixed fabric is obtained in which the cellulose acetate constituents are colored a deep red and the viscose constituents a navy blue, coupling on both the constituents being completed at a temperature of about 30° C.

15

*Example 4*

A cellulose acetate viscose fabric is dyed in a similar manner to that described in Example 3 using a bath containing the following constituents:

20

|                         | Per cent |
|-------------------------|----------|
| Fast red RL base        | 1        |
| Naphthol AS.LT          | 2        |
| Caustic soda            | 0.5      |
| 25 Diazo fast green GFL | 3        |

After treatment with the above liquor the fabric is introduced into a diazotising bath for about 30 minutes in which diazotisation is effected and coupling on the cellulose acetate constituents 30 takes place. The fabric is then rinsed and introduced into a bath containing 1% of phenyl-methyl-pyrozolone in which coupling on the viscose takes place.

In this manner a dyed mixed fabric is obtained 35 in which the cellulose acetate constituents are colored a bright red and the viscose constituents green.

In each of the above examples the fabric treated 40 contains about 50% of each type of yarn. In Examples 2-4 the proportions of dyestuffs are calculated on the weights of the respective yarns and the other reagents on the weights of the 45 fabrics, except where otherwise stated.

The process of the present invention is applicable 45 to the coloring of mixed yarns, fabrics and other textile materials containing constituents made of cellulose acetate or other organic derivative of cellulose together with other constituents, for example cotton or regenerated cellulose 50 fibres. The organic derivative of cellulose constituents may for example be continuous filaments, obtained for example by the extrusion of a solution of cellulose acetate, spun yarns, made from staple fibres obtained for example from 55 such continuous filaments or by the acetylation of cotton or other cellulosic fibres without destroying their structure, or filamentary materials of relatively high denier such as straw or slit foil. The process is applicable to the production 60 of any suitable azo dyestuffs on the mixed materials. As examples of suitable bases which may be employed may be mentioned o-chloraniline, para-nitraniline, para-nitrobenzene azo-para-xylyidine, m-nitro-p-toluidine, o-anisidine, di-anisidine,  $\alpha$ -naphthylamine, benzidine, and mono-aceto-acetyl-4,4'-diamino-azobenzene, while as examples of suitable coupling components may be mentioned resorcin,  $\beta$ -naphthol,  $\alpha$ -naphthol, amino-phenols and amino-naphthols, 65 oxy-naphthoic acids,  $\beta$ -naphthylamine, p-amino-diphenylamine, and  $\beta$ -keto-acetyl arylides, e. g. diaceto acetyl-o-tolidide.

Having described our invention, what we desire to secure by Letters Patent is:

75 1. Process for the coloration with azo dyestuffs

of mixed textile materials containing filaments, 10 yarns or the like of organic derivatives of cellulose and cellulosic filaments, yarns or the like, which comprises impregnating the materials with the diazotizable base component and the coupling component of the dyestuff for the organic derivative of cellulose constituent of the materials and with the diazotizable base component of the dyestuff for the cellulose derivative constituent of the materials, and then effecting diazotization 15 of the diazotized bases and the coupling of the coupling component for the cellulose derivative dyestuff, and then coupling with a coupling component of the dyestuff for the cellulose constituents.

2. Process for the coloration with azo dyestuffs 20 of mixed textile materials containing filaments, yarns or the like of cellulose acetate and cellulosic filaments, yarns or the like, which comprises impregnating the materials with the diazotizable base component and the coupling component of the dyestuff for the cellulose acetate constituent of the materials and with the diazotizable base component of the dyestuff for the cellulose constituent of the materials, and then 25 effecting diazotization of the diazotized bases and the coupling of the coupling component for the cellulose derivative dyestuff, and then coupling with a coupling component of the dyestuff for the cellulose constituents.

3. Process for the coloration with azo dyestuffs 30 of mixed textile materials containing filaments, yarns or the like of organic derivatives of cellulose and cellulosic filaments, yarns or the like, which comprises impregnating the materials with the diazotizable base component and the coupling component of the dyestuff for the organic derivative of cellulose constituent of the materials and with the diazotizable base component of the dyestuff for the cellulose constituents of the materials, then 35 diazotizing the base components, applying a coupling component for the dyestuff of the cellulose constituents and coupling the same at about room temperature, and subsequently effecting coupling of the components of the dyestuff for the organic derivative of cellulose constituent at a materially higher temperature.

4. Process for the coloration with azo dyestuffs 40 of mixed textile materials containing filaments, yarns or the like of cellulose acetate and cellulosic filaments, yarns or the like, which comprises impregnating the materials with the diazotizable base component and the coupling component of the dyestuff for the cellulose acetate constituent of the materials and with the diazotizable base component of the dyestuff for the cellulose constituent of the materials, then diazotizing the base components, applying a coupling component for the dyestuff of the cellulose constituents and coupling the same at about room temperature, and subsequently effecting coupling of the components of the dyestuff for the cellulose acetate constituent at a materially higher temperature.

5. Process for the coloration with azo dyestuffs 45 of mixed textile materials containing filaments, yarns or the like of cellulose acetate and cellulosic filaments, yarns or the like, which comprises impregnating the materials with the diazotizable base component and the coupling component of the dyestuff for the cellulose acetate constituent of the materials and with the diazotizable base component of the dyestuff for the cellulose constituent of the materials, then 50 diazotizing the base components, applying a coupling component for the dyestuff of the cellulose constituents and coupling the same at about room temperature, and subsequently effecting coupling of the components of the dyestuff for the cellulose acetate constituent at a materially higher temperature.

azotizing the base components, applying a coupling component for the dyestuff of the cellulosic constituents, and coupling same at 10 to 20° C., and thereafter effecting coupling of the components of the dyestuff for the cellulose acetate constituent at 60 to 80° C.

6. Process for the coloration with azo dyestuffs of mixed textile materials containing filaments, yarns or the like of organic derivatives of cellulose and cellulosic filaments, yarns or the like, which comprises impregnating the materials with the diazotizable base component and the coupling component of the dyestuff for the organic derivative of cellulose constituent of the materials, the said coupling component being an arylide of 2:3 hydroxynaphthoic acid, and with the diazotizable base component of the dyestuff for the cellulosic constituent of the materials, and then effecting diazotization of the diazotized bases and 20 the coupling of the coupling component for the cellulose derivative dyestuff, and then coupling with a coupling component of the dyestuff for the cellulosic constituents.

7. Process for the coloration with azo dyestuffs of mixed textile materials containing filaments, yarns or the like of cellulose acetate and cellulosic filaments, yarns or the like, which comprises impregnating the materials with the diazotizable base component and the coupling component of the dyestuff for the cellulose acetate constituent of the materials, the said coupling component being an arylide of 2:3 hydroxynaphthoic acid, and with the diazotizable base component of the dyestuff for the cellulosic constituent of the materials, then diazotizing the base components, applying a coupling component for the dyestuff of the cellulosic constituents and coupling the same at about room temperature, and subsequently 15 effecting coupling of the components of the dyestuff for the cellulose acetate constituent at a materially higher temperature.

GEORGE HOLLAND ELLIS. 20  
CHARLES FINLEY TOPHAM.